

# United States Patent [19]

Andrzajak et al.

[11] 3,809,146

[45] May 7, 1974

[54] **METHOD OF OPENING AN  
INTERMEDIATE VESSEL NOZZLE FOR  
CONTINUOUS CASTING**

3,581,948 6/1971 Detalle ..... 266/34 PP X  
3,684,267 8/1972 Andrzajak et al. ..... 266/38  
3,773,226 11/1973 Kutzer ..... 222/148

[75] Inventors: **Sigmund L. Andrzajak, Chicago,  
Ill.; Michael A. Orehoski, Duquesne;  
James T. Shapland, Wilkins  
Township, Allegheny County, both  
of Pa.; Raymond S. Szumilas,  
Chicago, Ill.**

[73] Assignee: **United States Steel Corporation,  
Pittsburgh, Pa.**

[22] Filed: **Feb. 18, 1972**

[21] Appl. No.: **227,476**

[52] U.S. Cl. .... **164/66, 164/82, 266/34 PP**

[51] Int. Cl. .... **B22d 11/10**

[58] Field of Search ..... **164/66, 82; 266/34 PP,  
266/38; 222/DIG. 13**

[56] **References Cited**

UNITED STATES PATENTS

3,320,053 5/1967 Lehman ..... 75/59

Primary Examiner—Robert D. Baldwin  
Attorney, Agent, or Firm—Ralph H. Dougherty

[57] **ABSTRACT**

A method of and apparatus for handling liquid steel in a tundish preparatory to teeming the steel into a continuous casting mold. Initially the tundish outlet is closed with a slidable gate which has a porous plug aligned with the outlet. Inert gas is injected into the steel through this plug to agitate the steel in the region of the tundish outlet. Inert gas injection is terminated shortly before the commencement of teeming, and oxygen rich gas is injected to react exothermically with the steel in the nozzle well area. Thereafter the porous plug slidable gate is replaced with a conventional gate having a teeming opening.

4 Claims, 1 Drawing Figure



PATENTED MAY 7 1974

3,809,146



## METHOD OF OPENING AN INTERMEDIATE VESSEL NOZZLE FOR CONTINUOUS CASTING

In the continuous casting of steel, molten metal is poured from a ladle into an intermediate pouring vessel, such as a tundish or a degassing vessel, and thence into a water-cooled mold. The refractory lining of the intermediate vessel is usually recessed above the nozzle, and the nozzle is closed by a refractory closure member, such as a sliding gate. The metal that first reaches this recess has already lost much of its heat to the refractory lining of the vessel. This rather quiescent metal settles into the recess, loses additional heat to the surrounding refractory and begins to solidify. The molten metal in the vessel above the recess does not contain sufficient superheat to remelt the solidified metal. Opening the blocked recess heretofore has necessitated the use of an oxygen lance, which is an undesirable practice as it may impair the quality of the metal and damage refractories of the intermediate vessel. Whenever pouring is interrupted by closing the nozzle, molten metal in the recess above the nozzle cools more rapidly than the metal above it because it has a larger surface area in contact with the surrounding refractory, that is, it has a higher surface-to-volume ratio. The cooling action of the refractory can result in the formation of frozen steel or "skull" in the nozzle region and prevent stream flow when the nozzle is reopened. The present invention affords a method of preventing a recess from blocking, either before pouring begins or when pouring is interrupted.

It is known that inert gases can be introduced to molten metal to provide various treatments. For example, gas may be insufflated through a porous plug in a sliding gate to stir molten metal within a vessel. However, practices used heretofore have not successfully overcome the problem of failure of gates to open properly.

It is the principle object of our invention to provide a method of insuring the full opening of a nozzle of an intermediate vessel, such as a tundish, to assure a proper pouring stream.

It is also an object of our invention to provide a method of opening a nozzle of an intermediate vessel, regardless of whether such nozzle is totally or partially blocked by solidified metal.

The single FIGURE is a partly diagrammatic cross section through the nozzle of a bottom-pour intermediate vessel equipped with a sliding gate which employs a permeable refractory block in the gas passageway beneath the vessel nozzle and includes our gas-injection apparatus.

Vessel 10 has a refractory lining 11 for receiving molten metal. The bottom wall of the vessel has a well or recess 12 and an outlet opening 13 and carries a refractory nozzle plate 14 fixed to its underside aligned with the opening. A sliding gate closure member 15 is mounted beneath the nozzle plate. The gate can be supported and operated in any desired manner, hence, we have not shown the supporting and operating mechanism. The gate includes a solid refractory block 16, a surrounding steel jacket 17, and a gas-permeable refractory plug 18 centered in the upper portion of block 16. A pipe 19 is affixed at its upper end to jacket 17 which forms with plug 18 a cylindrical gas distribution chamber 20. Pipe 19 extends to sources 21 and 22 of inert gas and oxygen rich gas respectively, either of which can be admitted thereto through a three-way

valve 23. If jacket 17 is made of more than one piece, it must be tightly welded to prevent any gas leaks, either through the jacket itself or between the jacket and pipe 19.

In the continuous casting of steel, especially in a multistrand operation, about 60 seconds elapse from the time the vessel begins to fill until it is desirable to commence pouring at least one strand. While the vessel is filling, we introduce inert gas (usually argon) through the porous plug 18 to agitate the molten metal in the nozzle well area. Between five and fifteen seconds before we are ready to cast one strand, we operate valve 23 to change the flow through the porous plug from inert gas to oxygen-rich gas, preferably commercially pure oxygen. The oxygen flow rate is from 5 to 15 standard cubic feet per minute. The steel in the well area is superheated about 2°F for each cubic foot of oxygen injected into the steel. The oxygen reacts exothermically with the molten metal, removing any skull present in the nozzle well. Immediately after oxygen injection, we replace gate 15 with a gate 24 which has a pouring opening 25 and commence the casting operation.

We prefer to use an oxygen flow rate of from 8 to 10 cubic feet per minute for a period of 7 to 10 seconds. As a specific example, in utilizing our method on a four-strand tundish, we have injected argon, which is a coolant to the steel, into the nozzle well for up to 4 minutes, then introduced commercially pure oxygen for just 10 seconds at 8 cubic feet per minute and obtained a free-flowing stream having good stream characteristics.

The foregoing conditions are critical for the successful practice of our invention. A flow rate of oxygen of less than 5 cubic feet per minute or for a time of less than 5 seconds does not insure that a nozzle will open. Conversely, a flow rate greater than 15 cubic feet per minute of oxygen or for a time greater than 15 seconds overheats the steel, and upon teeming the metal into the mold, the steel may melt the chill pins in the mold stool on contact. Thus, when downward movement of the starter bar is initiated, the mold stool will separate from the casting and the entire heat may be lost. Further, excessive oxygen oxidizes the carbon in the steel to carbon dioxide, causing it to leave the steel as a gas. When elements that form oxides in the steel are lost, the solidification rate is reduced and breakouts below the mold are not only common, but are almost certain.

Porous plug 18 in sliding gate 15 must have a diameter which is less than that of the orifice in nozzle plate 14, and the axis of plug 18 should coincide with the axis of the nozzle plate orifice. Preferably the nozzle in plate 14 is made of zirconia, which is only effective to about 3,000°F, above which temperature it will become eroded. Oxygen flow through the molten metal in this region will burn out the zirconia insert if the uppermost diameter of the porous plug is equal to or greater than that of the opening of the zirconia insert.

Prior to our invention, it was necessary to preheat the nozzle well to about 2,400°F to insure sufficient heat in the well to prevent the freezing of steel at the beginning of introduction of steel to the intermediate vessel. Unexpectedly, our invention has made it totally unnecessary to preheat the nozzle well.

Although the drawing shows a porous plug gate used on a single nozzle intermediate vessel, it is even more

advantageously used in accordance with our invention on a multiple-nozzle vessel.

It can readily be seen from the foregoing that we have invented a method of opening the nozzle of an intermediate vessel at any time, regardless of whether such nozzle is blocked by solidified metal.

We claim:

1. A method of handling liquid steel in an intermediate vessel in preparation for teeming the steel into a continuous-casting mold, said method comprising:

- a. closing the outlet of the vessel with a slidable gate which has a porous plug aligned with the outlet;
- b. introducing liquid steel to the vessel;
- c. injecting inert gas to the steel in the vessel through said plug to agitate the steel while it is introduced until shortly before teeming is to begin;
- d. terminating inert gas injection within about 15 seconds of the time teeming is to begin;

e. injecting at least enough oxygen-rich gas at a rate of 5 to about 15 scfm into the steel in the vessel through said plug for a period of from 5 to about 15 seconds immediately after termination of inert gas injection to superheat the steel in the region of the outlet and remove any skull which has formed; and

f. immediately opening the gate and teeming the steel from the vessel into the mold at the conclusion of the step of injecting oxygen-rich gas.

2. A method according to claim 1 wherein said oxygen-rich gas is commercially pure oxygen.

3. A method according to claim 2 wherein oxygen is injected at a rate of 8 to 10 scfm.

4. A method according to claim 2 wherein oxygen is injected through said plug for a period of from 7 to 10 seconds.

\* \* \* \* \*

20

25

30

35

40

45

50

55

60

65

UNITED STATES PATENT OFFICE  
CERTIFICATE OF CORRECTION

Patent No. 3,809,146 Dated May 7, 1974

Inventor(s) Sigmund L. Andrzejak et al.

It is certified that error appears in the above-identified patent and that said Letters Patent are hereby corrected as shown below:

The first inventor's name should read

-- Sigmund L. Andrzejak --.

Signed and sealed this 29th day of October 1974.

(SEAL)

Attest:

McCOY M. GIBSON JR.  
Attesting Officer

C. MARSHALL DANN  
Commissioner of Patents